

## UNITED STATES PATENT OFFICE.

ERNST AEUER, OF BERLIN, GERMANY, ASSIGNOR TO GENERAL ELECTRIC COMPANY,  
A CORPORATION OF NEW YORK.

## MAKING TUNGSTEN FILAMENTS.

1,191,552.

Specification of Letters Patent. Patented July 18, 1916.

No Drawing.

Application filed August 10, 1910. Serial No. 576,522.

*To all whom it may concern:*

Be it known that I, Dr. ERNST AEUER, a subject of the King of Prussia, residing at Berlin, Germany, have invented certain new and useful Improvements in Making Tungsten Filaments, of which the following is a specification.

My invention relates to the manufacture of tungsten filaments, and its object is to facilitate the sintering of the filaments.

Hitherto when making tungsten filaments for electric incandescence lamps it has been customary to make a pasty mass from the raw material with or without an organic or inorganic binder and to press the filaments from the mass or to squirt them through dies. From these raw filaments the binder is removed, and if tungsten compounds has been taken as raw material, it is also necessary to reduce the compounds. Besides, the filaments must be sintered, which may be performed immediately after the just mentioned processes and jointly with them or separately. Filaments produced in this way are inferior to drawn metal filaments as regards mechanical qualities. This may be explained by the supposition, that the smallest particles of a drawn metal wire are in such degree intimately connected one with another by the melting processes passed by the metal before being drawn to wire, as it never can be attained by the paste-processes. Besides, if the paste has been made with a binder, the latter being driven out before or during the sintering breaks up the structure of the pressed filament in such degree, that the metal particles, which are to be sintered, are in a relatively loose connection and that, therefor, the sintering of the single particles materially is rendered more difficult.

The last mentioned inconvenience is especially marked, if the sintering of the filaments is not effected by current introduced into them, but is achieved in an electric furnace in an atmosphere of hydrogen, for example in a carbon tube furnace, into which the filaments are brought on supports of oxid of thorium. In this case when sintering it is not possible to raise the temperature as high, as if the filaments are sintered by current flowing through them, as the furnace, then, would deteriorate too rapidly and must be renewed very frequently.

The invention purposes to facilitate the

sintering of the filaments by a preparatory treatment in order that it may be attained in an electric furnace in an atmosphere of hydrogen without endangering the furnace too much. For this purpose the tungsteniferous filaments are subjected before the sintering to a chemical reaction, which brings the separate molecules in connection by glowing the filaments in ammonia-gas or in another gas containing nitrogen or in such a gas mixture at a relatively low temperature and by converting them, thereby, into a nitrogen compound. The filaments must be heated to at least noticeable red-heat, it is advisable to employ a temperature of 700-900° centigrade. By the following heating up to bright incandescence which is to be performed in order to sinter the filaments in the furnace in an atmosphere of hydrogen the nitrogen compound is decomposed again.

A suitable gas for the preparatory treatment is especially a mixture of ammonia-gas and hydrogen or of nitrogen and hydrogen. If the trioxid of tungsten or other oxygen compounds have been taken as raw material, by the glowing in the just mentioned gases the reduction of the oxygen compound may be effected, too. The elimination of the binder or of the carbon left in the filament from the binder may also be joined with the described heating process in the gas containing nitrogen by first raising the temperature as high, as is necessary for the elimination of the carbon, and then lowering the temperature to about 700-900° centigrade. It is however equally possible to remove the binder or its carbon earlier or later.

The conversion of the filaments in the nitrogen compound may be effected wholly or partly. As trials show, by the described processes the later sintering is facilitated and filaments of greater mechanical strength are produced.

One could mind to perform the sintering, too, in the above mentioned gas or gas mixture instead of in hydrogen by raising the temperature up to bright incandescence after the formation of the nitrogen compound. This is however not practical, as at the high temperature the nitrogen of the gas attacks the carbon tube of the furnace with production of cyanogen, whereby the persons

charged with the performance of the processes would easily be exposed to dangers. Even with the employment of a furnace consisting of a high melting metal inconvenience would result, as the ammonia-gas would diffuse in the outer room through the metal tube. On the other hand it is not practical to perform the preparatory treatment above described in such a mixture of hydrogen and 10 nitrogen or hydrogen and ammonia-gas, which is poor in nitrogen, as in this case the conversion of the filaments in the nitrogen compound would require a long time. From this it may be seen how advantageous it is 15 to employ two different gases, viz. a gas rich in nitrogen during the preparatory treatment and hydrogen during the sintering.

What I claim as new and desire to secure by Letters Patent of the United States, is—  
20 1. The method of manufacturing tungsten filaments which consists in heating a filament comprising an oxygen compound of tungsten in an atmosphere rich in nitrogen to a temperature at which said filament is 25 converted into a nitrogen compound and then decomposing said compound by heating to a materially higher temperature in hydrogen, to decompose the nitrogen com-

pound and sinter the resulting tungsten metal.

2. The method of manufacturing tungsten filaments which consists in converting filaments comprising an oxygen compound of tungsten into a nitrogen compound of tungsten by heating the same in a nitrogen-containing gas to a temperature of about 30 700 to 900° C., and then heating said filaments by radiant heat to a temperature of 35 bright incandescence in hydrogen to decompose the nitrogen compound and sinter the 40 resulting tungsten filaments.

3. In a process for the manufacture of tungsten filaments the step which consists in heating filaments containing an oxygen compound of tungsten to a red heat in an atmosphere of ammonia to bring the metallic particles into intimate connection and then decomposing the resulting nitrogen compound to yield a metallic filament.

In witness whereof, I have hereunto set 50 my hand this 26th day of July, 1910.

DR. ERNST AEUER.

Witnesses:

JULIUS RUMLAND,  
OSKAR SINGER.

Copies of this patent may be obtained for five cents each, by addressing the "Commissioner of Patents, Washington, D. C."